

## UNITED STATES PATENT OFFICE

1,945,221

## PRINTING OF TEXTILE FIBERS

Sebastian Gassner and Hermann Berthold,  
Leverkusen-on-the-Rhine, Germany, assignors  
to General Aniline Works, Inc., New York, N. Y.,  
a corporation of Delaware

No Drawing. Application May 19, 1930, Serial  
No. 453,855, and in Germany May 29, 1929

27 Claims. (Cl. 8—5)

The present invention relates to improvements in the printing of cotton with vat or sulfur dye-stuffs.

In accordance with the invention cotton is printed according to any desired method with printing pastes of vat or sulfur dyestuffs containing besides the different ingredients, known for the preparation of such printing pastes, an alkali metal salt of an unsubstituted sulfonic or carboxylic acid of the benzene or naphthalene series or, a hydrogenation product thereof, or a benzene or naphthalene sulfonic acid substituted by alkyl groups or dialkylamino groups, or a benzene or naphthalene carboxylic acid, substituted by alkyl-, hydroxy-, or dialkylamino groups.

It may be mentioned that the term "printing pastes" is intended to include all kinds of pastes usually applied for cotton printing purposes, such pastes for example as are obtainable by mixing vat dyestuffs with thickenings, water, glycerine or another similar water soluble alcohol, potassium carbonate, sodium carbonate, sodium formaldehyde sulfoxylate, sodium hydrosulfite or a mixture of the latter with sodium formaldehyde sulfoxylate and the like. The alkali metal salts of the sulfonic or carboxylic acids above specified may be added to the printing pastes at any stage of the preparation of the same. The printing of cotton with said printing pastes may be performed in the usual manner, for example, with the aid of a printing engine, whereupon the printings are dried to a certain extent, steamed with wet steam (e. g. in a Mather-Platt) and developed by oxidation, e. g., with an aqueous solution of an alkali metal bichromate and acetic acid, rinsed and soaped while boiling. It will also be possible to use the pastes containing the sulfonic or carboxylic acids above specified in slop-padding processes, and it may be mentioned that the best results are generally obtained when working with pastes which are reduced only on the fiber while steaming, which pastes generally do not contain hydrosulfites, but, e. g., sodium formaldehyde sulfoxylate as the reducing agent.

Numerous advantages result from the presence of the alkali metal salts mentioned in the printing of cotton. In the first place it is possible in this manner to obtain concentrated dyestuff pastes, which do not settle or separate even on prolonged storing; in the second place it is frequently possible to obtain dyestuff powders of a high degree of dryness, which can be worked up immediately to very uniform printing pastes; thirdly, the addition of the alkali metal salts described above produces in most cases a considerable strengthening of the printings obtainable, which strengthening amounts in some cases to 40% and which by far exceeds the action of sodium benzylaniline sulfonate, or other similar

salts which are known as additions to printing pastes.

As alkali metal salts of the kind above referred to may be mentioned by way of example:

Alkali metal salts of benzoic acid, ortho-toluic acid, salicylic acid, phthalic acid, benzene sulfonic acid, para-toluene sulfonic acid, naphthalene-alpha- and beta-sulfonic acid, dialkyl-aniline sulfonic acids, such as sodium dimethyl- or diethyl-metanilate, sodium dimethylsulfanilate, sodium dimethyl-2-toluidine-4-sulfonate, furthermore, the sodium salt of cyclohexane carboxylic acid, sodium tetrahydronaphthalene-beta-sulfonate and so on. One or more of such salts may be added to the dyestuff preparations with a good effect.

The following examples will illustrate our invention without restricting it thereto:

## Example 1

A. 20 parts by weight of 6,6'-dichloro-4,4'-dimethylbisthio-naphthene-indigo (in form of an aqueous paste)

15 parts by weight of the sodium salt of dimethylmetanilic acid

40 parts by weight of glycerine

are evaporated in a plain pan until the paste has a dyestuff content of 18%. The dyestuff preparation thus obtainable is of permanent durability, does not settle as the aqueous paste, neither freezes nor dries up and does not form crusts. The sodium salt of dimethylmetanilic acid can be replaced, for example, by the sodium salts of dimethyl-sulfanilic acid, benzoic acid, salicylic acid, ortho-cresotinic acid, naphthalene-alpha- and beta-monosulfonic acid, tetrahydro-naphthalene-beta-sulfonic acid and the like.

B. 10 parts by weight of the dyestuff preparations thus obtainable are mixed with

10 parts by weight of water and

80 parts by weight of a thickening containing in

100 parts by weight

6 parts by weight of wheat starch

6 parts by weight of British gum powder

16 parts by weight of gum 1:1

17 parts by weight of tragacanth 65:1000

10 parts by weight of glycerine

15 parts by weight of potassium carbonate

15 parts by weight of sodium formaldehyde sulfoxylate and

15 parts by weight of water.

The printing pastes thus obtainable are used for printing purposes in the ordinary manner. The printings are steamed whilst moist, devel-

oped with potassium chromate-acetic acid and soaped while boiling. The printings produced in this manner on cotton are considerably more powerful than those obtainable by the same directions but without the addition of the alkali metal salts mentioned.

C. 20 parts by weight of the dyestuff preparations according to A.

- 10 10 parts by weight of glycerine
- 10 2 parts by weight of sodium-benzylaniline sulfonate
- 15 15 parts by weight of potassium carbonate
- 15 12 parts by weight of sodium formaldehyde sulfoxylate
- 15 41 parts by weight of a thickening containing in
- 15 100 parts by weight
- 20 35 parts by weight of British gum powder
- 20 13 parts by weight of wheat starch
- 20 2 parts by weight sodium benzyl aniline sulfonate
- 20 50 parts by weight water

25 are used for printing in the same manner as under B.

*Example 2*

- 30 20 parts by weight of the finely divided dyestuff, obtainable in accordance with example 1 of British Patent No. 15,607/07 from naphtho-oxythiophen-carboxylic acid, in form of an aqueous paste
- 35 15 parts by weight of sodium benzene sulfonate and
- 35 40 parts by weight of glycerine

40 are evaporated on the water bath with stirring until a paste of 20% dyestuff content is obtained. The dyestuff preparation thus obtainable does not dry up and can be worked up immediately by the customary processes to printing pastes, which on printing, for example, according to the process mentioned in Example 1, B., yield more powerful printings than are obtainable without the addition of sodium benzene sulfonate.

*Example 3*

- 50 3 parts by weight of a 60% dyestuff powder obtainable by drying
- 579 parts by weight of a 10.33% paste of the dyestuff obtained in accordance with Example 1 of U. S. Patent No. 1,667,848, in the presence of
- 55 2 parts by weight of calcined sodium carbonate and
- 38 parts by weight of the sodium salt of dimethyl-metanilic acid in an enamelled drying dish on the water bath or on a roller dryer, heated by means of steam at 1½-2 atmospheres pressure or by some other means, are mixed for printing purposes with
- 60 17 parts by weight of water and
- 80 parts by weight of a thickening as described in Example 1, B. The printings obtainable with this paste in the usual manner are without stippling, they are fixed better and show a strengthening of shade compared with the printing obtainable according to the same method but without the addition of the sodium salt of dimethylmetanilic acid.

*Example 4*

- 3 parts by weight of a 60% dyestuff powder, obtainable by drying 484 parts by weight of an aqueous paste of the dyestuff specified in Example 1, together with 80 parts by weight of the sodium salt of dimethyl-metanilic acid and
- 2 parts by weight of sodium carbonate in the manner described in Example 3, are used for printing purposes as described in Example 3. The printings on cotton even in printing processes without previous reduction are considerably stronger than the printings obtainable from a normal aqueous paste of the same dyestuff material without the addition of the sodium salt of dimethylmetanilic acid.

*Example 5*

- 30 parts by weight of the dyestuff of Example 1 in form of an aqueous paste
- 19 parts by weight of the sodium salt of dimethylmetanilic acid
- 0.5 parts by weight of sodium carbonate and
- 0.5 parts by weight of sodium isobutynaphthalenesulfonate (as wetting agent) are evaporated to dryness in the manner described in Example 3. The powder is finely ground and sieved and can be used without further treatment for printing in the manner described in Example 3.

The sodium salt of dimethylmetanilic acid can also be replaced by the sodium salt of dimethyl-10-toluidine-4-sulfonic acid.

*Example 6*

- 30 parts by weight of the dyestuff specified in Example 1, in form of an aqueous paste
- 18 parts by weight of the sodium salt of tetrahydro-naphthalene-beta-sulfonic acid and
- 2 parts by weight of sodium carbonate are worked up to a dry dyestuff preparation, as described in Example 3 and display the same advantages in printing as described in the preceding examples.

*Example 7*

- 30 parts by weight of 3,3'-dichloro-N-dihydro-1,2-2',1'-anthraquinone-azine (in the form of an aqueous paste)
- 18 parts by weight of the sodium salt of tetrahydro-naphthalene-beta-sulfonic acid and
- 2 parts by weight of sodium carbonate are evaporated to dryness. The dyestuff powder thus obtainable is finely ground and used for printing purposes according to Example 1, B. The dyestuff preparation yields printings without stippling, which are fixed more quickly than those obtainable by employing a normal aqueous paste of the same dyestuff without the addition of sodium tetrahydronaphthalene sulfonate.

*Example 8*

When the dyestuff specified in Example 1 is replaced by flavanthrone and sodium benzene sulfonate is used instead of sodium dimethyl-metanilate, a preparation likewise yielding stronger printings is obtained.

*Example 9*

When the dyestuff specified in Example 1 is replaced by that described in Example 1 of Brit. Patent 246,683 as 3,4-9,8-dibenzopyrene-5,10-quinone and sodium benzene sulfonate is used instead of sodium dimethylmetanilate, a preparation likewise yielding stronger printings than a normal aqueous paste of the same dyestuff without the addition of sodium benzene sulfonate, is obtained.

*Example 10*

In Example 1 the dyestuff can be replaced by 15 dimethoxy-dibenzanthrone (Color Index page 265 No. 1101) and as the addition sodium salicylate or sodium dimethylmetanilic acid can be used, in which case dyestuff preparations valuable in cotton printing are likewise obtained.

20

*Example 11*

When the dyestuff specified in Example 9 is replaced by that of the German Patent No. 25 242,621, a preparation likewise yielding stronger printings is obtained.

*Example 12*

30 From the dyestuff obtainable according to Example 3 (first dyestuff) of British Patent No. 201,786, glycerine, and the sodium salt of diethylmetanilic acid or the sodium salt of ortho-toluylic acid, dyestuff preparations can be produced in accordance with Examples 1 or 2, said dyestuff preparations also yielding especially 35 strong printings.

*Example 13*

40 From the dyestuff known in the literature (Scholl, Berichte der deutschen Chemischen Gesellschaft Vol. 43, page 349) as pyranthrone, in combination with the sodium salt of naphthalene-beta-sulfonic acid or dimethylmetanilic acid or dimethyl-2-toluidine-4-sulfonic acid 45 valuable printings are obtainable in accordance with the method described in Example 1.

50

*Example 14*

The printing capacity of the dyestuff specified in Brit. Patent No. 23179/03 is improved by the addition of, for example, the sodium salt of cyclohexane carboxylic acid, the sodium salt of tetrahydronaphthalene-beta-sulfonic acid, the sodium salt of naphthalene-alpha- or beta-sulfonic acid.

60

*Example 15*

179 parts by weight of an aqueous paste containing 11% of 6,6'-diethoxy-2,2'-bisthionaphtheneindigo (Color Index No. 62 1217)  
40 parts by weight of crude glycerine 88%  
15 Parts by weight of the sodium salt of benzene sulfonic acid  
55 are evaporated until the paste shows a dyestuff content of 15%. The printings obtainable with this dyestuff preparation on cotton are stronger and the fixing process is much shortened compared with printings obtainable by employing a normal aqueous paste of the same dyestuff not containing sodium benzene sulfonate.

*Example 16*

356.5 parts by weight of an aqueous paste containing 11.2% of the dyestuff obtained from bromo-1-chloro-2,3-naphthoisatin 80 and 4-methoxy-1-naphthol in accordance with the example of Brit. Patent No. 289,154

40 parts by weight of glycerine and 10 parts by weight of the sodium salt of di- 85 methylmetanilic acid

are concentrated until the paste again shows a dyestuff content of 11.2%.

*Example 17*

20 parts by weight of 4,7,4'-7'-tetramethyl- 90 5,5'-dichlorobisthionaphthene indigo (in the form of an aqueous paste)

40 parts by weight of crude glycerine 15 parts by weight of the sodium salt of ben- 95 zene sulfonic acid

are concentrated to a dyestuff content of 17%.

The dyestuff preparations obtainable in accordance with the last examples also display, when used for printing purposes after working up to printing pastes in any desired manner, the 100 valuable properties already described.

We claim:

1. Process which comprises printing cotton with a printing paste comprising a vat dyestuff and 105 an alkali metal salt of a compound of the group consisting of unsubstituted sulfonic and carboxylic acids of the benzene and naphthalene series, hydrogenation products thereof, benzene and naphthalene sulfonic acids substituted by 110 alkyl groups or dialkylamino groups, and benzene or naphthalene carboxylic acids substituted by alkyl-, hydroxy- or dialkylamino groups.

2. Process which comprises printing cotton with printing pastes comprising a vat dyestuff 115 and an alkali metal salt of an unsubstituted benzene- or naphthalene-sulfonic acid.

3. Process which comprises printing cotton with printing pastes comprising a vat dyestuff and an alkali metal salt of a dialkylamino benzene sulfonic acid. 120

4. Process which comprises printing cotton with printing pastes comprising a vat dyestuff and an alkali metal salt of a dimethylamino benzene sulfonic acid. 125

5. Process which comprises printing cotton with printing pastes comprising a vat dyestuff and an alkali metal salt of benzene sulfonic acid.

6. Process which comprises printing cotton with printing pastes derived from vat dyestuffs, 130 said pastes comprising an alkali metal salt of tetrahydronaphthalene sulfonic acid.

7. Vat dyestuff preparations consisting of a vat dyestuff, water, glycerine and an alkali metal salt of a compound of the group consisting of unsubstituted sulfonic and carboxylic acids of the benzene and naphthalene series, hydrogenation products thereof, benzene and naphthalene sulfonic acids substituted by alkyl groups or dialkylamino groups, and benzene or naphthalene 135 carboxylic acids substituted by alkyl-, hydroxy- or dialkylamino groups.

8. Vat dyestuff preparations consisting of a vat dyestuff, water, glycerine and an alkali metal salt of an unsubstituted benzene or naphthalene 140 sulfonic acid.

9. Vat dyestuff preparations consisting of a vat dyestuff, water, glycerine and an alkali metal salt of a dialkylamino benzene sulfonic acid.

10. Vat dyestuff preparations consisting of a 150

vat dyestuff, water, glycerine and an alkali metal salt of a dimethylamino benzene sulfonic acid.

11. Vat dyestuff preparations consisting of a vat dyestuff, water, glycerine and an alkali metal salt of benzene sulfonic acid.

12. Vat dyestuff preparations consisting of a vat dyestuff, water, glycerine and an alkali metal salt of tetrahydronaphthalene sulfonic acid.

13. Printing pastes suitable for printing cotton, which comprise a vat dyestuff, a thickening and an alkali metal salt of a compound of the group consisting of sulfonic and carboxylic acids of the benzene and naphthalene series, hydrogenation products thereof, benzene and naphthalene

15 sulfonic acids substituted by alkyl groups or dialkylamino groups, and benzene and naphthalene carboxylic acids substituted by alkyl-, hydroxy- or dialkylamino groups.

14. Printing pastes suitable for printing cotton, which comprise a vat dyestuff, a thickening and an alkali metal salt of an unsubstituted benzene or naphthalene sulfonic acid.

15. Printing pastes suitable for printing cotton, which comprise a vat dyestuff, a thickening and an alkali metal salt of a dialkylamino benzene sulfonic acid.

16. Printing pastes suitable for printing cotton, which comprise a vat dyestuff, a thickening and an alkali metal salt of a dimethylamino benzene sulfonic acid.

17. Printing pastes suitable for printing cotton, which comprise, a vat dyestuff, a thickening and an alkali metal salt of benzene sulfonic acid.

18. Printing pastes suitable for printing cotton, which comprise a vat dyestuff, a thickening and an alkali metal salt of tetrahydronaphthalene sulfonic acid.

19. The process which comprises printing cotton with a printing paste comprising 6.6'-dichloro-4.4'-dimethyl - bisthionaphthene indigo, and an alkali metal salt of a compound selected from the group consisting of dimethylmetanilic acid, dimethylsulfanilic acid, dimethylsulfanilic acid and salicyclic acid.

45

80

20. The process which comprises printing cotton with a printing paste comprising the dyestuff obtainable from naphtho-oxythiophene carboxylic acid by oxidation with potassium ferric cyanide in caustic soda solution, and an alkali metal salt of benzene sulfonic acid.

21. The process which comprises printing cotton with a printing paste comprising 3.3'-dichloro-N-dihydro-1.2.2'.1'-anthraquinone azine and an alkali metal salt of tetrahydronaphthalene-beta-sulfonic acid.

22. A printing paste comprising 6.6'-dichloro-4.4' - dimethylbisthionaphthene indigo and an alkali metal salt of a compound selected from the group consisting of dimethylmetanilic acid, dimethyl-sulfanilic acid and salicylic acid.

23. A printing paste comprising the dyestuff obtainable from naphtho-oxythiophene carboxylic acid by oxidation with potassium ferric cyanide in caustic soda solution, and an alkali metal salt of benzene sulfonic acid.

24. A printing paste comprising 3.3'-dichloro-N-dihydro-1.2.2'.1'-anthraquinone azine and an alkali metal salt of tetrahydronaphthalene-beta-sulfonic acid.

25. A vat dyestuff preparation consisting of 6.6'-dichloro-4.4'-dimethyl-bisthionaphthene indigo, water, glycerine and an alkali metal salt of a compound selected from the group consisting of dimethyl-metanilic acid, dimethylsulfanilic acid and salicylic acid.

26. A vat dyestuff preparation consisting of the dyestuff obtainable by reacting upon naphthoxythiophene-carboxylic acid with potassium ferric cyanide in caustic soda solution, water, glycerine and an alkali metal salt of benzene sulfonic acid.

27. A vat dyestuff preparation consisting of 3.3'-dichloro-N-dihydro-1.2.2'.1'-anthraquinone azine, water, glycerine, and an alkali metal salt of tetrahydronaphthalene-beta-sulfonic acid.

95

100

105

110

115

120

50

125

55

130

60

135

65

140

70

145

150

SEBASTIAN GASSNER.  
HERMANN BERTHOLD.